

## 1

3,025,960

ELECTROSTATIC CONCENTRATION OF  
MINERALS

Charles C. Cook, Salt Lake City, Utah, assignor to International Minerals & Chemical Corporation, a corporation of New York.  
No Drawing. Filed Sept. 23, 1960, Ser. No. 57,892  
20 Claims. (Cl. 209—3)

This invention relates to the electrostatic concentration of minerals. More particularly, the invention relates to the restoration of charge susceptibility to fractions of minerals which have been rendered non-responsive, to charging *inter alia* by contact electrification.

Various procedures for the electrostatic concentration of minerals differentially charged primarily by contact electrification are described in Lawyer Patents 2,805,769 and 2,847,147, LeBaron Patent 2,738,875, and elsewhere in the art. Such mineral concentration techniques frequently yield middling, concentrate or tail fractions unresponsive to further significant differential charging. Expedients such as elevated temperatures and agitation effective initially to insure a charge differential appropriate for effective electrostatic separation are ineffective when applied to such charge non-responsive fractions. Accordingly, conventional procedures such as recycle of the non-responsive fractions to the dry head feed or the direct subjection such fractions to additional stages of electrostatic treatment are ineffective to achieve significant additional beneficiation.

Various procedures have been suggested for the restoration of charge susceptibility to non-responsive fractions resulting from prior passage of a mineral mixture through an electrostatic field. One such procedure described in Lawyer Patent 2,723,029, entails exposing clean surfaces predominantly by surface attrition of the particles of the non-responsive fraction. An alternative procedure described in Lawyer Patent 2,805,770 contemplates mixture of non-responsive fractions with materials of a different work function. Yet another expedient disclosed in Lawyer Patent 2,832,469, contemplates washing of such non-responsive fractions followed by drying of the washed fractions.

It is apparent that the various expedients suggested in the prior art for the restoration of charge susceptibility to electrostatically separated mineral fractions each entail serious economic disadvantages inherent in the cost of attrition grinding, the provision, separation and recycle of materials of different work function, washing and drying and the like.

It is accordingly a primary object of this invention to provide a novel method effective to restore charge susceptibility to mineral fractions separated by electrostatic concentration.

It is a more specific object of the invention to provide a novel method effective to restore charge susceptibility to electrostatically separated fractions of relatively soft, attritionable minerals, such as phosphate rock.

It is another object of the invention to provide an improved electrostatic mineral beneficiation procedure having particular applicability to phosphate rock.

It is also a specific object of the invention to provide a novel technique for the electrostatic concentration of minerals under conditions such that the mineral undergoes no significant charge modification while in the electrostatic field.

It is an additional object of the invention to provide a method of restoring charge susceptibility to unagentized charge non-responsive mineral mixtures.

It is more particularly an object of the invention to provide an improved method for the electrostatic concentration of minerals in which the initial head feed, at

## 2

one stage is wet, and a non-responsive fraction resulting from electrostatic concentration is recycled to such wet head feed and thereby again rendered susceptible to differential charging.

5 In accordance with this invention, a wet head feed comprising an ore comminuted to liberation is dried, differentially charged and introduced into an electrostatic field to produce a concentrate fraction and at least one other fraction of impaired response to differential charging requisite to a further stage of electrostatic concentration, said other fraction is recycled to and commingled with said wet head feed to impart effective charge susceptibility to said fraction and said mixture of wet head feed and recycled fraction is differentially charged, and beneficiated by passage through an electrostatic field.

10 It will be appreciated that the invention differs fundamentally from techniques predicated upon chemical reagent treatment to insure effective differential charging. Such a procedure is described; for example, in Johnson Patent 2,197,865, which describes the recycle of an electrostatic middling to a reagentizing operation in which the head feed is concurrently treated.

15 The invention is generically applicable to the electrostatic concentration of all minerals, including without limitation, all metallic and nonmetallic, silicate and non-silicate ores. Representative minerals include hematite, the various iron ores, copper ores, mercury ores, uranium ores, and the other metallic ores, phosphate rock, calcitic phosphate ores, lithium ores such as spodumene, 20 the various feldspar ores, oil shale, and the like. The invention is particularly applicable to the beneficiation of phosphate rock ores such as Florida pebble phosphate.

25 The invention is also generically applicable in combination with all of the various techniques known to be useful in electrostatic mineral concentration. A preferred expedient entails heating the feed mineral mixture to the electrostatic concentration step to a temperature of at least 150° F., but below the decomposition point of any component of said mixture, inducing the heated mineral mixture to accept differential charges while at a temperature of at least 150° F. and passing the differentially charged mixture through an electrostatic field while at a temperature of at least 150° C. Such processes are described in respect to contact electrification 30 charging and so-called free fall electrostatic separation 35 in Lawyer Patent 2,805,769, the disclosure of which is incorporated herein by reference.

40 It will be appreciated that the process of the invention is embractive of the separation of particulate mineral mixtures in electrostatic fields of all types and without regard to the nature or physical structure of the apparatus utilized. A preferred form of apparatus is of the "free-fall" type which comprises spaced stationary electrodes of opposite signs such as is disclosed, for example, 45 in FIGURE 3 of the Lawyer Patent 2,805,769.

45 The process of the invention, however, may also be practiced in roll-type separators such as disclosed in Johnson Patent 2,197,865, in which the electrodes take the form of a rotating, relatively large diameter roll by which the particles of the materials to be separated are 50 conveyed into the field, and a relatively smaller electrode spaced from the roll. In respect to those minerals, which are mixtures of nonconductors, the actual separation occurs in such roll separators in substantially the same way as in "free-fall" apparatus utilizing stationary electrodes. 55 Such a result is a consequence of the fact that the nonconducting mineral particles are effectively charged substantially entirely by contact electrification rather than by inductive conduction from the roll surface of a roll separator as in the case of conductor particles.

60 70 The invention preferably is practiced under conditions which effect no significant change in the charge on the

particles undergoing separation during passage through the electrostatic field, as would be occasioned, for example, by electron spray.

The invention generically contemplates electrostatic fields of any strength requisite, as may readily be determined by a person skilled in the art, to effect the desired separation between the charged particles. Generally the field gradient or strength may vary from about 1,000 volts to about 15,000 volts per inch of distance between the electrodes. It is preferred to utilize a total applied potential difference of 30,000 to 250,000 volts maintained in a form of uniform potential substantially free of alternating components. Filtered direct current low in alternating current ripple is appropriately utilized. Rectified radio frequency power supplies are also appropriate.

In general, the particle size of the mixtures separated in accordance with the invention should fall within the range of from about 4 to about 200 mesh, preferably from about 8 to about 100 mesh. In general, comminution of ores to a commercially practical degree of liberation is suitable. Removal of fines may be desirable but is not essential.

The conventional preparation of Florida pebble phosphate for the free fall electrostatic separation of apatite from silica is described *inter alia*, in Lawver Patent 2,805,769. Such preparation entails washing, desliming and comminution to liberation. Accordingly, the invention in a preferred embodiment of the invention as applied to Florida pebble phosphate entails washing, desliming, and comminution to produce, as a head feed, a wet substantially liberated phosphate pebble ore comprising a mixture of phosphate and silica particles, drying and heating sand mixture to a temperature of at least about 150° F., differentially charging the phosphate and silica particles in said mixture while at a temperature of at least 150° F., passing the differentially charged mixture through an electrostatic field to produce a concentrate fraction and at least one other fraction of impaired response to further differential charging, and recycling at least a portion of said charge non responsive fraction of said wet head feed. Preferably the mixture of particulate phosphate and silica is charged and passed through the electrostatic field at a temperature of from about 350° F. to about 550° F.

The step of drying phosphate ores in preparation for differential charging and electrostatic concentration preferably entails substantial agitation in a first stage to effect high heat transfer and a minimum of agitation in a final stage to improve the response of the dried ore to charging particularly by contact electrification. Such drying techniques are described in Lawyer Patent 2,847,123.

The fraction of impaired charge susceptibility appropriately comprises of from about 2% to about 80% and preferably from about 10% to about 50% by weight of the solids, in the mixture of said fraction with the wet head feed. The specific percent of recycle material in the wet admixture depends, in general, on the operating conditions and the composition of the fresh feed.

The invention will be more fully understood from the following example.

## EXAMPLE

Florida pebble phosphate obtained as washer debris having a size range of from -1 millimeter to +150 mesh after having been through the usual desliming operation in a classifier for flotation plant beneficiation was de-watered and dried.

The dried solids, which had a BPL content of 27.4% by weight, were delivered to a vibrating trough for discharge of the particles as freely falling bodies between the electrodes of an electrostatic separation unit having the electrodes spaced approximately 10 inches apart and maintained at a potential gradient of approximately 9000 volts per inch.

A tail fraction from this first stage was passed through

a second or so-called "scavenger" stage of separation, and a scavenger concentrate and a tail were separately recovered. The scavenger concentrate analyzed 48.84% BPL. The result from passing the scavenger concentrate through a third stage of electrostatic separation are given below in Table 1.

Table 1

|     | Pan Numbers | Weight percent | Percent BPL |
|-----|-------------|----------------|-------------|
| 10  |             |                |             |
| 1-3 |             | 24.2           | 19.28       |
| 4   |             | 32.8           | 46.83       |
| 5   |             | 29.6           | 65.80       |
| 6-8 |             | 13.4           | 69.28       |

From the previous listed data, it may be noted that 62.4 weight percent was in the center pans (4 and 5) which indicates that this material was substantially non-responsive to the electrostatic field.

In a series of tests, various amounts of the scavenger concentrate were recycled and mixed with the wet solids from the classifier which has a water content of about 18%. The wet mixtures were dried at 300° F. for two hours, charged and subjected to an electrostatic beneficiation operation as above described. The amount of scavenger concentrate mixed with the fresh feed was varied as indicated in Table II.

Table II

| Test No. | Wt. percent Fresh Feed | Wt. percent Scavenger Concentrate | Pan No. | Wt. percent | Percent BPL |
|----------|------------------------|-----------------------------------|---------|-------------|-------------|
| 30       |                        |                                   |         |             |             |
| 35       |                        |                                   |         |             |             |
| 1        | 100                    | 0                                 | 1-3     | 41.3        | 3.39        |
|          |                        |                                   | 4       | 17.9        | 11.66       |
|          |                        |                                   | 5       | 13.2        | 44.81       |
|          |                        |                                   | 6-8     | 27.6        | 66.72       |
|          |                        |                                   | 1-3     | 42.5        | 2.69        |
|          |                        |                                   | 4       | 15.5        | 10.67       |
| 40       | 90                     | 10                                | 5       | 13.4        | 50.68       |
| 2        |                        |                                   | 6-8     | 28.6        | 68.51       |
|          |                        |                                   | 1-3     | 39.6        | 2.29        |
| 3        | 80                     | 20                                | 4       | 14.8        | 11.36       |
|          |                        |                                   | 5       | 12.6        | 50.09       |
|          |                        |                                   | 6-8     | 33.0        | 69.01       |
|          |                        |                                   | 1-3     | 40.5        | 3.08        |
| 4        | 70                     | 30                                | 4       | 13.4        | 15.44       |
|          |                        |                                   | 5       | 14.5        | 55.96       |
| 45       |                        |                                   | 6-8     | 31.6        | 70.68       |
| 5        | 60                     | 40                                | 1-3     | 36.6        | 3.30        |
|          |                        |                                   | 4       | 13.7        | 20.27       |
|          |                        |                                   | 5       | 19.3        | 56.51       |
|          |                        |                                   | 6-8     | 30.4        | 69.79       |
|          |                        |                                   | 1-3     | 27.8        | 3.90        |
| 50       | 6                      | 40                                | 4       | 9.6         | 31.44       |
|          |                        |                                   | 5       | 25.8        | 51.44       |
|          |                        |                                   | 6-8     | 36.8        | 61.61       |
|          |                        |                                   | 1-3     | 24.2        | 19.28       |
| 7        | 0                      | 100                               | 4       | 32.8        | 46.83       |
|          |                        |                                   | 5       | 29.6        | 65.80       |
|          |                        |                                   | 6-8     | 13.4        | 69.24       |

Analogous results are affected with the other ores contemplated by the invention and with each of the various types of apparatus with which the invention may be practiced.

Having now fully described and illustrated the invention, what is desired to be secured and claimed by Letters Patent is set forth in the appended claims.

1. A process for the electrostatic concentration of minerals without chemical reagentizing consisting essentially of providing a wet head feed of an ore comminuted to liberation, drying said head feed, imparting a differential charge to the particulate value and gangue components of said dried head feed, introducing said differentially charged particles into an electrostatic field to produce a concentrate fraction and at least one other fraction of impaired response to differential charging requisite to a further stage of electrostatic concentration, forming a mixture of said other fraction with said wet head feed to impart effective charge susceptibility thereto, drying, and differentially charging said mixture, and beneficiating

said dried and charged mixture by passage through an electrostatic field.

2. The process of claim 1 wherein said head feed and said mixture are differentially charged by contact electrification.

3. The process of claim 2 wherein said dried and differentially charged head feed is passed as freely falling bodies through said electrostatic field to produce said concentrate fraction and said other fraction.

4. The process of claim 3 wherein said mixture is 10 beneficiated by passage through said electrostatic field as freely falling bodies.

5. The process of claim 1 wherein said head feed is subjected to an electron spray, and said concentrate fraction and said other fraction are produced by passage of said head feed through a roll-type electrostatic separator.

6. The process of claim 5 wherein said mixture is charged by an electron spray and said mixture is beneficiated by passage through a roll-type separator.

7. The process of claim 1 wherein said ore is a phosphate ore.

8. The process of claim 1 wherein said ore is Florida pebble phosphate.

9. The process of claim 1 wherein said ore is an iron ore.

10. The process of claim 1 wherein said ore is hematite.

11. The process of claim 1 wherein said ore is comminuted to liberation at a mesh size of from about eight to about one hundred.

12. A process for the electrostatic concentration of phosphate rock ore without chemical reagentizing consisting essentially of washing, desliming and comminuting said ore to provide as a head feed, a wet mixture of phosphate and silica particles, drying and heating said mixture to a temperature of at least 150° F., differentially charging the phosphate and silica particles in said mixture while at a temperature of at least 150° F., passing the differentially charged mixture into an electrostatic field while at a temperature of at least 150° F. to produce a concentrate fraction and at least one other fraction of

impaired response to further differential charging, and recycling said other fraction to said wet head feed.

13. The process of claim 12 wherein phosphate and silica particles in said mixture are differentially charged by contact electrification.

14. The process of claim 12 wherein said phosphate and silica particles in said mixture are differentially charged and passed into said electrostatic field at a temperature of from about 350° F. to about 550° F.

15. The process of claim 12 wherein said other fraction is recycled in an amount requisite to constitute from about two percent to about eighty percent of the total weight of the solids in the mixture of said fraction with said head feed.

16. The process of claim 12 wherein said other fraction is recycled in an amount requisite to constitute from about ten percent to about fifty percent of the total weight of the solids in the mixture of said fraction with said head feed.

17. The process of claim 12 wherein said differentially charged mixture of phosphate and silica particles is passed through said electrostatic field as freely falling bodies.

18. The process of claim 12 wherein said differentially charged mixture of phosphate and silica particles is conveyed into said electrostatic field by a rotating roll of a roll-type electrostatic separator.

19. The process of claim 12 wherein the field gradient of said electrostatic field is from about 1000 volts to 30 about 15,000 volts per inch of distance between the electrodes.

20. The process of claim 12 wherein the differential charge on the phosphate and silica particles is not significantly changed during passage through said electrostatic field.

References Cited in the file of this patent

UNITED STATES PATENTS

40 2,197,865 Johnson ----- Apr. 23, 1940  
2,805,769 Lawyer ----- Sept. 10, 1957